

E. G. GILSON.  
PROCESS OF MAKING BEARING COMPOSITIONS.  
APPLICATION FILED JULY 7, 1910.

1,071,044.

Patented Aug. 26, 1913.



*Metal and Graphite*

Witnesses:

*Marcus L. Byng.*  
*Carl G. Klock.*

Inventor:

Emery G. Gilson,  
by *Alfred H. Davis*  
His Attorney.

# UNITED STATES PATENT OFFICE.

EMERY G. GILSON, OF SCHENECTADY, NEW YORK, ASSIGNOR TO GENERAL ELECTRIC COMPANY, A CORPORATION OF NEW YORK.

## PROCESS OF MAKING BEARING COMPOSITIONS.

1,071,044.

Specification of Letters Patent. Patented Aug. 26, 1913.

Application filed July 7, 1910. Serial No. 570,787.

To all whom it may concern:

Be it known that I, EMERY G. GILSON, a citizen of the United States, residing at Schenectady, county of Schenectady, State 5 of New York, have invented certain new and useful Improvements in Processes of Making Bearing Compositions, of which the following is a specification.

My invention relates to the manufacture 10 of metallic articles containing a lubricating material, such as graphite, and which are suitable for uses requiring a minimum of friction between rubbing or sliding parts, such as brushes for dynamo-electric 15 machines, dash-pots, bearings for shafts and the like.

In accordance with my invention, an intimate mixture of graphite and a reducible metallic compound or compounds, for example, metallic oxids, is heated to a temperature sufficient to reduce all but a small percentage of the oxids by interaction with some of the graphite. The reduction mass, still containing a certain percentage of unreduced material, is then compressed into desired form and the reduction is continued after compression until it is substantially complete and consolidation of the metals has taken place. The presence of unreduced 25 material in the mixture before compression appears to prevent both segregation and agglomeration of the metal powder and results in a homogeneous, strong product in which the graphite is distributed with great uniformity. Although appearing perfectly 30 solid and dense, articles made by this process are still porous enough to absorb considerable oil.

The accompanying drawing illustrates a 40 dynamo-electric machine brush made in accordance with my invention.

I will explain my invention as applied to the manufacture of metallic articles consisting chiefly of copper associated with 45 some metal or metals, which will alloy with copper, such as tin, lead or zinc, and in addition to these metals containing graphite as a lubricating material. The alloying metal is added to aid the consolidation of the 50 copper particles by soldering them together during the final stage of the process to form

a coherent homogeneous mass, and it also acts as a lubricant.

A typical mixture, for example, consists of 100 parts of black copper oxid, CuO, 10 55 parts of tin oxid, SnO<sub>2</sub>, and 125 parts of graphite. These materials, of course, should be in a finely divided condition and thoroughly mixed. For this purpose they can conveniently be pulverized in a ball mill. 60 This mixture is placed in a suitable retort, consisting for example of copper, and is heated for about 8 hours to a temperature of 650 to 700° C. At the end of this time a large part of the metals will have been reduced by the graphite to a metallic state 65 but the mixture should contain small amounts of unreduced oxids. The amount of unreduced material will vary somewhat with the character of the mixture. Some 70 mixes need contain at this stage of the proceedings no more than .5 to 2.5% of oxid but, of course, only relative figures can be given. The length of time that the mixture is heated and the temperature to which it is 75 subjected should be varied in accordance with the character and proportion of the mixture and other conditions so as to leave at least the above amount of unreduced oxid. For example, if lead is used in addition to 80 tin, the reduction temperature should not be much more than 600° C. and the time should be shortened.

Upon cooling, the mixture is put through a 100 mesh sieve and is compressed into pre-determined form—for example, the block 1 as shown in the drawing. The compressed articles are then packed in charcoal, so as to exclude air, and are again heated to a temperature of 650 to 700° C. until the reduction 90 of the metals is substantially complete and alloyage between the copper and tin, lead, or other metal has taken place. To obtain these results, it is advisable to regulate the heat and the duration of heating so as to 95 reach the above temperature at the end of about 18 hours, the heating being then continued for about 60 hours. If the finished article is to be used as a brush it may then be provided with suitable current connections 100 2.

As an alternative method of obtaining the

thorough incorporation of the materials, a 5  
reducible salt, for example, copper acetate is  
dissolved in water and the tin oxid and  
graphite are added to the solution. The so-  
lution is evaporated to dryness, the tin oxid  
and graphite being maintained uniformly  
distributed by constant stirring. The mass  
is then placed in a ball mill and finely  
powdered.

10 The subsequent reduction is preferably car-  
ried out in a crucible which is provided with  
a dasher for the purpose of constantly agi-  
tating the material during the reduction.  
The agitation in this case appears to be  
15 necessary to avoid agglomeration of the  
metal. The reduction takes place at a tem-  
perature in the neighborhood of 600° C.,  
the range of temperature being somewhat  
lower than is the case when employing cop-  
20 per oxid. The reduction is continued for 2½  
to 3½ hours, at the end of which time all  
but about 5% of the tin oxid and copper  
oxid formed at this stage should have been  
reduced to the metallic state by the graphite.  
25 The copper, of course, will not be present  
as acetate since the acetate is decomposable  
by heat and breaks down to form the oxid.  
In this case, as well as in the alternative  
method of preparation described above,  
30 the mixture will be spoiled by carrying the  
reduction too far. In the latter method,  
however, the minimum amount of unre-  
duced oxid permissible is in the neighbor-  
hood of 2½%, and as a rule 5% is preferable.  
35 After reduction the powder is put through  
a 100 mesh sieve and compressed into the  
required form. The pressed blocks are  
finally heated for a long time in order to  
complete the reduction and agglomerate the  
40 particles in the manner described above.

These examples will serve to indicate the  
steps of the process, but it will, of course,  
be understood that the proportions will be  
varied in accordance with the properties de-  
45 sired in the finished article, the length of  
time required for reduction and the tem-  
perature of the reduction being in turn  
varied somewhat in accordance with the ma-  
terials used and their proportion, but in  
50 each case the conditions should be so regu-  
lated as to leave a small amount of unre-  
duced metallic oxid in the reduction mix-  
ture before compressing the same into final  
form.

55 Articles made by the above process are  
more or less porous and are capable of ab-  
sorbing as high as 5% by weight of oil.  
Whether any oil can be introduced advan-  
tageously into the finished article, of course,  
60 depends upon the use to which they are  
finally put.

It is to be understood that my invention  
applies to the manufacture of bearing ma-  
terial containing metals other than those

above specified. Any metal which has the 65  
requisite physical properties and which can  
be readily reduced, as, for example silver,  
can be used in place of copper. In the same  
manner other alloying metals can be used,  
or they may be left out entirely. 70

What I claim as new and desire to secure  
by Letters Patent of the United States, is,—

1. The process which consists in subject-  
ing a mixture of reducible metallic com-  
pounds with a reducing material to a tem-  
perature sufficient to reduce by the action  
of said reducing material all but a small  
percentage of said compounds to the metal-  
lic state, then compressing the mixture in a  
predetermined shape and finally heating at 80  
the reduction temperature until the reduc-  
tion is substantially complete.

2. The process which consists in subject-  
ing a mixture of copper oxid, an oxid of  
metal alloyable with copper and graphite 85  
to a temperature at which reduction of said  
oxids by the graphite takes place and con-  
tinuing the reduction until all but a small  
percentage of the metallic constituents have  
been reduced, then compressing the mixture 90  
and continuing the reduction until said  
metals have been substantially completely  
reduced and alloyage has taken place.

3. The process of making current col-  
lectors for dynamo-electric machines which 95  
consists in subjecting to a temperature of  
about 600° to 700° C. a mixture of graphite,  
copper oxid, and an oxid of a reducible  
metal capable of alloying with copper and  
continuing the reduction until all but a 100  
small percentage of the metals have been  
reduced, then compressing the mixture and  
subsequently continuing the reduction.

4. The process which consists in subject-  
ing a mixture of copper oxid, tin oxid and 105  
graphite to a temperature of about 600 to  
700° C., until all but about .5-5% of said  
oxids have been reduced to the metallic  
state, then compressing the mixture and  
subsequently continuing the reduction until 110  
it is substantially complete.

5. The process which consists in subject-  
ing a mixture of reducible metallic com-  
pound and a reducing agent to the tem-  
perature necessary to effect chemical reac- 115  
tion, agitating the material while reduc-  
tion takes place, molding the reduction  
mixture before the reduction is complete  
and then continuing the reduction until con-  
solidation of the materials has taken place. 120

6. The process of making a metal-graphite  
composition which consists in molding a  
mixture comprising copper, a soft metal  
alloyable with copper and reducible by  
carbon from its oxid, a small percentage of 125  
an oxid of at least one of said metals, and  
graphite in excess of the amount necessary  
to reduce said oxid, and heating in an inert

environment until substantial reduction of the oxid and consolidation of the materials has taken place.

7. The process of making brushes for dynamo electric machines which consists in compressing a mixture comprising copper, tin, about .5 to 5% of oxid of said metals, and graphite in excess of the amount necessary to reduce said oxid, and firing the

molded mass with the exclusion of air until substantial reduction of the oxid and agglomeration and alloyage has taken place.

In witness whereof, I have hereunto set my hand this 6th day of July, 1910.

EMERY G. GILSON.

Witnesses:

HELEN ORFORD,  
BENJAMIN B. HULL.